

## [54] PROCESS FOR THE DECARBURIZATION OF MOLTEN METAL

[75] Inventors: **Edwin Francis Bauer**, Niagara Falls; **Roger Nels Dokken**, Katonah; **Robert Amos Hard**, Lewiston; **Umesh Kumar Malhotra**, Peekskill, all of N.Y.

[73] Assignee: **Union Carbide Corporation**, New York, N.Y.

[22] Filed: **Nov. 1, 1971**

[21] Appl. No.: **194,454**

[52] U.S. Cl. .... **235/151.12**, 75/60, 444/1

[51] Int. Cl. .... **C21d 3/04**, G06f 15/46

[58] Field of Search. .... 235/150.1, 151, 151.1, 235/151.12; 75/59, 60, 133; 23/230, 253; 444/1

## [56] References Cited

## UNITED STATES PATENTS

|           |        |                       |           |
|-----------|--------|-----------------------|-----------|
| 3,046,107 | 7/1972 | Nelson et al. ....    | 75/59     |
| 3,169,058 | 2/1965 | Nelson ....           | 75/133    |
| 3,252,790 | 5/1966 | Krivosky ....         | 75/60     |
| 3,329,495 | 7/1967 | Ohta et al. ....      | 75/60     |
| 3,377,158 | 4/1968 | Mayer et al. ....     | 75/60     |
| 3,463,631 | 8/1969 | Vayssiere et al. .... | 75/60     |
| 3,528,800 | 9/1970 | Blum et al. ....      | 235/151.1 |

|           |         |                          |            |
|-----------|---------|--------------------------|------------|
| 3,561,743 | 2/1971  | Schroeder et al. ....    | 75/60      |
| 3,565,606 | 2/1971  | Carlson et al. ....      | 75/60      |
| 3,594,155 | 7/1971  | Ramachandran ....        | 75/60      |
| 3,621,217 | 11/1971 | Carr et al. ....         | 235/151.12 |
| 3,614,682 | 10/1971 | Smith ....               | 235/151.12 |
| 3,619,174 | 11/1971 | Fujii et al. ....        | 75/60      |
| 3,754,895 | 8/1973  | Ramachandran et al. .... | 75/60      |

Primary Examiner—Felix D. Gruber  
Attorney, Agent, or Firm—Eugene Lieberstein

## [57] ABSTRACT

A process for making steel by refining a predetermined mass of molten metal having a composition containing at least carbon and iron comprising: injecting oxygen into such mass with a gaseous diluent at a first dilution ratio and calculating from the activity coefficient of each element in the mass a theoretical equilibrium partial pressure of carbon monoxide for the oxidation reaction of each element; calculating the absolute maximum partial pressure of carbon monoxide; selecting the lowest partial pressure and calculating a new metal analysis for the mass; changing the dilution ratio upon meeting a given criterion and repeating the process until the carbon level of the mass has dropped to a predetermined level.

45 Claims, 8 Drawing Figures





FIG. I

INVENTORS  
EDWIN F. BAUER  
ROBERT A. HARD  
ROGER N. DOKKEN  
UMESH K. MALHOTRA  
BY *Eugene L. Lichtenstein*  
ATTORNEY



**FIG. 2**

INVENTORS  
EDWIN F. BAUER  
ROBERT A. HARD  
ROGER N. DOKKEN  
UMESH K. MALHOTRA  
BY *Signs here*  
ATTORNEY



FIG. 2a

INVENTORS  
 EDWIN F. BAUER  
 ROBERT A. HARD  
 ROGER N. DOKKEN  
 UMESH K. MALHOTRA

BY   
 ATTORNEY

PATENTED JUN 11 1974

3,816,720

SHEET 4 OF 8

FRACTION OF THE AOD VESSEL  
WORKING LINING AFFECTED BY  
THERMAL VARIATIONS



FIG. 3

INVENTORS  
EDWIN F. BAUER  
ROBERT A. HARD  
ROGER N. DOKKEN  
UMESH K. MALHOTRA

BY

*George S. Schuster*  
ATTORNEY

PATENTED JUN 11 1974

3,816,720

SHEET 5 OF 8



FIG.4

INVENTORS  
EDWIN F. BAUER  
ROBERT A. HARD  
ROGER N. DOKKEN  
UMESH K. MALHOTRA  
BY *Ernest Leibman*  
ATTORNEY



FIG. 5

## INVENTORS

EDWIN F. BAUER  
ROBERT A. HARD  
ROGER N. DOKKEN  
UMESH K. MALHOTRA

BY *James R. Schmitz*  
ATTORNEY



FIG. 6

INVENTORS

EDWIN F. BAUER  
ROBERT A. HARD  
ROGER N. DOKKEN  
UMESH K. MALHOTRA

BY

  
ATTORNEY



FIG. 7

INVENTORS  
 EDWIN F. BAUER  
 ROBERT A. HARD  
 ROGER N. DOKKEN  
 UMESH K. MALHOTRA

BY *Roger Hard*  
 ATTORNEY

## PROCESS FOR THE DECARBURIZATION OF MOLTEN METAL

### BACKGROUND OF THE INVENTION

This invention relates to a method of decarburizing molten metal in the refining of steel.

When steel is decarburized with oxygen, equilibrium is established among the metals, the carbon and oxygen at the particular temperature and pressure. Such equilibrium determines the extent to which carbon can be removed, without oxidizing metallics, chromium in particular, from the melt. It is now well recognized that the thermodynamic activity in the bath and the equilibrium established among the elements and the evolved gaseous atmosphere may be modified by dilution of the oxygen with an inert gas.

The limit to which the temperature may be elevated is based upon both practical and economic considerations relating to the effect of high temperatures on the life of the vessel lining as well as on the life of the tuyeres which are necessary for injecting the oxygen and inert gas directly into the melt from beneath its surface. On the other hand, dilution of the blowing oxygen with inert gas also involves economic considerations since it decreases the rate of steel production in proportion to the percent volume of inert gas introduced, not to mention the cost of the inert gas itself, which can be substantial.

Heretofore, the principle concern was to reduce the carbon content of the molten bath to a specified level while minimizing the oxidation loss of other elements. Other than the desire to prevent the rapid deterioration of the refractory, by careful temperature surveillance, the process was conducted at the expense of relatively slow steel production rate and without regard to the quantity of inert gas utilized. The apparent lack of concern with economics was justified on the basis that it was impossible to sample the bath periodically during a production run to determine the extent of metallic oxidation and actual bath temperature. It was considered far wiser to insure an acceptable end melt composition than to risk making an off grade heat by increasing the rate of production and conserving inert gas. At the very best, certain generalized guidelines were empirically established, through actual experience, for changing the dilution ratio at fixed time intervals and at an assumed temperature condition for a specific melt using a given refractory lining composition.

### OBJECTS OF THE INVENTION

It is an object of the present invention to provide a process for decarburizing a mass of molten metal in terms of achieving from knowledge of only the initial mass composition, weight and temperature, a predetermined end composition under the most favorable economic conditions.

It is another object of the present invention to provide a method for optimizing, in terms of combined performance and economics, the decarburization of a mass of molten metal to consistently yield final melt composition and temperature which conforms to a desired specification for such melt and at a relatively high rate of production.

### SUMMARY OF THE INVENTION

The process of the present invention is based on the theoretical assumption that for any small interval of

time the oxygen combines with carbon until sufficient pressure of carbon monoxide is generated that further combination of oxygen with carbon is precluded by the preference of oxygen for that metallic element the reduction of whose oxide produces the lowest equilibrium partial pressure of carbon monoxide. From such assumption a theoretical mathematical model has been developed for calculating, at given selected intervals of time, the lowest equilibrium partial pressure of carbon monoxide from which a new mass composition, weight and temperature of the melt can be determined and from which, either automatically or through an operator, readjustments may be made in the dilution ratio to optimize the process. The mathematical model simulates the complicated natural processes occurring in the refractory lined vessel in terms of the reaction thermodynamics, heat and mass balances and thus predicts the process of a heat. Although, the mathematical calculations may be made by a person; in practice, it could not be done quickly enough to be useful, and therefore the present process requires a computer for its practical implementation.

In its broadest aspects, the present invention is a method for refining steel by controlling the decarburization of a predetermined mass of molten metal comprising carbon and iron contained within a refractory lined vessel having means for injecting oxygen and a diluting gas into the mass and adjustable gas flow control means for varying the flow rate of the gases; wherein the process comprises:

- a. setting the adjustable control means to establish a first flow rate greater than zero for oxygen and a first flow rate for the diluting gas;
- b. utilizing a computer to carry out the following sequence of steps:
  1. calculating, a plurality of activity coefficients, from data corresponding to the initial flow rate setting of each gas respectively and from the initial composition, weight and temperature of the mass of metal, that define the thermodynamic activities of each element in the mass as a function of the composition of the mass, each coefficient reflecting the activity of each element in terms of the percentage of the element and the dependency of the element on the percentage of the other elements in the mass, with the activity of iron being equal to its mole fraction and wherein the activities of the oxides of each element have predetermined values;
  2. calculating a theoretical equilibrium partial pressure of carbon monoxide for the oxidation reaction of each element by means of the coefficients at the given temperature;
  3. calculating the absolute maximum partial pressure of carbon monoxide assuming all the oxygen injected reacted solely with the carbon;
  4. selecting the lowest theoretical equilibrium partial pressure of carbon monoxide from (2) and comparing such with the absolute maximum partial pressure of carbon monoxide from (3);
  5. make a determination as to whether the lowest theoretical equilibrium partial pressure has a magnitude greater than the absolute maximum partial pressure and from said determination if such theoretical partial pressure is greater than the absolute maximum partial pressure than further calculate using said first gas flow rates, the

- amount of carbon oxidized and a new metal analysis and temperature for the composition.
6. make a determination as to whether the lowest theoretical equilibrium partial pressure has a magnitude of less than such absolute maximum partial pressure and from said determination if such theoretical partial pressure is of a magnitude lower than the absolute maximum partial pressure then further calculate from the theoretical equilibrium partial pressure of carbon monoxide and from said first gas flow rates the amounts of carbon and metal oxidized, a new metal analysis and temperature for the composition.
  7. providing an indication of said new carbon content in said mass;
  8. comparing the amount of oxidation of a specific signal element in the mass with a preestablished limit of oxidation for the specific element;
  9. providing an indication for resetting the adjustable gas flow control means to increase the proportion of diluting gas should the amount of oxidation of the specific element be at least equal to the preestablished limit of oxidation;
  - c. resetting the adjustable gas flow control means in accordance with the indication provided in step (9)
  - d. repeating the sequence from step (1) at predetermined time intervals of less than 2 minutes until the carbon content indicated in step (7) has at least decreased to a predetermined level.

#### BRIEF DESCRIPTION OF THE DRAWINGS

Advantages of the invention will be apparent from the following detailed description of the invention taken in conjunction with the following drawings in which:

FIG. 1 is a general schematic diagram of a decarburization system which utilizes the present invention;

FIGS. 2 and 2a combined represent the logic diagram of the preferred program for carrying out the present invention;

FIG. 3 is a graph, empirically established which defines the factor F for that portion of the refractory lined vessel which participates in the heat capacity of the system;

FIG. 4 is a graph showing the steady state temperature loss in the bath as a function of the size of the bath;

FIG. 5 is a graph, empirically established, which defines an acceptable band of bath temperature values for corresponding carbon contents.

FIG. 6 is a graph, empirically established, showing an alternative acceptable temperature range for corresponding carbon levels in the bath.

FIG. 7 is a simplified logic diagram of the preferred program shown in FIGS. 2 and 2a illustrating an alternative embodiment for changing the dilution ratio of oxygen in response to satisfying a given one of a number of different criteria.

#### DETAILED DESCRIPTION OF THE PROCESS

Shown diagrammatically in FIG. 1 is a simplified refining system for decarburizing steel consisting of a refractory lined refining vessel 10 charged with a predetermined mass of molten metal 12. The starting composition of the mass may represent essentially iron and

carbon where the refined end product is to be a low carbon iron. Alternatively, the starting composition for a stainless steel may be composed essentially of iron, carbon and chromium with nickel in some cases and with additional minor alloying constituents such as, for example, silicon and manganese. Moreover, for a nickel based alloy the starting composition may be composed essentially of carbon, iron, nickel, chromium, molybdenum and niobium. This invention is not to be construed as limited to any specific steel starting composition nor is the original percentage of any ingredient critical to the invention.

Oxygen is passed from a source (not shown) through an oxygen flow control 18 which regulates the flow rate of oxygen before injection into vessel 10. Likewise, a diluting inert gas is passed from a separate source (not shown) through a flow control 20 which regulates the flow of inert gas. The gas flow controls 18 and 20 respectively are conventional controllers which may be either automatically or manually operated as will as explained hereafter. The gases are combined in the mixing valve 16 and injected directly into the melt 12 preferably through a tuyere assembly 14. Other suitable gas injectors may be employed such as ceramic tubes, conduits, nozzles and the like so long as such means can withstand the bath temperatures involved without introducing undesirable contaminants. Separate means (not shown) may be used to control pressure in the respective flow lines.

The diluting gas may be any gas inert with respect to decarburization and preferably one selected from the group consisting of helium, neon, argon, krypton and xenon, or mixtures thereof. Nitrogen may also be used but with caution because of possible side effects. Argon is the most preferred gas.

The production rate as measured by the time required for decarburization is primarily affected by the temperature and gas flow rates and may be maximized by blowing the heat at the maximum total gas flow rate obtainable for the refining vessel and heat size, which is roughly 1,000 to 2,000 cubic feet per hour of total gas flow per ton of metal refining capacity for the vessel, and by keeping the flow rate of oxygen high relative to the flow rate of inert gas until the refractory is threatened by high temperature or until oxidation of the constituents in the melt other than carbon exceed predetermined levels. The temperature must also be kept above a minimum allowable temperature so that the heat can be finished, tapped and teemed into ingot molds without danger of solidifying prematurely. The present invention does not contemplate the use of temperature control elements or devices. Increases in temperature are due to the oxidation reactions occurring in the bath whereas reductions in temperature are due to absorption of heat by the applied inert gas, bath additions, and from the steady state heat loss occurring as a function of bath size, the heat capacity of the refractory and the vessel surroundings.

The method of the present invention whereby the gas flow controls 18 and 20 are operated, either manually or automatically, through the use of the digital computer to achieve optimum performance at maximum efficiency will now be described. The computer 22 is a general purpose computer which is programmed to operate in accordance with the logic diagram of FIGS. 2 and 2a representing the preferred embodiment of the present invention. Any programmer skilled in such art

can rapidly prepare a computer program in the language receptive to the computer utilized to operate in accordance with such logic diagram. In order to carry out the program the computer 22 must have stored in memory data representative of the mathematical equations taught herein as well as data representative of Appendixes A, B, and C and FIGS. 3, 4, and 5 or 6 respectively. The only input information necessary for any given heat is the starting metal composition, temperature, metal weight, the selected initial oxygen and inert gas flow rates and the final desired carbon content. From steelmaking experience it is known that an oxygen flow rate more than ten times greater than the inert gas flow rate will be harmful to the vessel tuyere assembly 14. Hence, as a practical matter the initial oxygen to inert gas flow rate should be less than 10 : 1.

Using the initial information the computer 22 calculates a plurality of coefficients that define the thermodynamic activities of each constituent element in the bath as a function of the composition of the bath. Employing such coefficients the computer 22 calculates the carbon monoxide partial pressure in equilibrium with carbon and the various metallic elements and their oxides. The reaction which produces the lowest equilibrium partial pressure of carbon monoxide is assumed to be favored and to proceed for some small increment of time. This increment of time is approximated for purposes of the present invention to be a period necessarily greater than zero but less than 2 minutes with a preferred range of between 3 to 30 seconds. Hence, the computer 22 without feedback can provide updated simulated sampling of the progress of a heat to determine whether and to what extend readjustment is to be made in the dilution ratio of oxygen and inert gas. The new conditions determined by the computer are automatically fed into memory and used in place of the previous conditions for the next iteration.

Upon injection, oxygen reacts immediately with some metallic species which, in turn, will react with dissolved carbon to form carbon monoxide according to the general reaction:



Where:  $M$  is any metallic element in the bath 12 such as Fe, Cr, Mn, Si, etc; C is Carbon; O is Oxygen and  $x$  and  $y$  are integers which represent the chemical formula of the metallic oxide in question.

The equilibrium constant for this general reaction can be calculated from the following equation:

$$K = \exp \Delta F^\circ / (-RT)$$

Where:  $K$  = equilibrium constant;  $\Delta F^\circ$  = standard free energy of the reaction;  $R$  is the gas constant and  $T$  = temperature ( $^{\circ}K$ ). The general chemical reaction represents reactions involving, for example, silicon, manganese, chromium, iron, nickel and/or other metallics which may be present in the mass. The appropriate equilibrium constants are calculated for each reaction in accordance with the above equation using the data from Appendix A as shown below.

#### APPENDIX A

##### Standard Free Energies of the Various Reactions of Interest

|   |                                                                                                                                                                                                                                                                                  |                                                                                                                                                    |
|---|----------------------------------------------------------------------------------------------------------------------------------------------------------------------------------------------------------------------------------------------------------------------------------|----------------------------------------------------------------------------------------------------------------------------------------------------|
| 5 | $\frac{1}{4}Cr_3O_4 = \frac{3}{4}Cr + O$<br>$\frac{1}{4}Cr_3O_4 + C = \frac{3}{4}Cr + CO(g)$<br>$\frac{1}{2}SiO_2 = \frac{1}{2}Si + O$<br>$\frac{1}{2}SiO_2 + C = \frac{1}{2}Si + CO(g)$<br>$MnO = Mn + O$<br>$MnO + C = Mn + CO(g)$<br>$FeO = Fe + O$<br>$FeO + C = Fe + CO(g)$ | 61,200 - 27.4T<br>56,925 - 37.24T<br>69,675 - 27.5T<br>65,400 - 37.34T<br>58,400 - 25.98T<br>54,125 - 35.82T<br>28,900 - 12.15T<br>24,175 - 21.99T |
|---|----------------------------------------------------------------------------------------------------------------------------------------------------------------------------------------------------------------------------------------------------------------------------------|----------------------------------------------------------------------------------------------------------------------------------------------------|

The theoretical partial pressure of carbon monoxide in equilibrium with carbon and the other ingredients in the bath may now be calculated from the following equation using the reactions given in Appendix B as set forth hereinbelow:

$$K = a_M^{x/y} P_{CO}^e / a_M^{1/y} a_C a_C$$

Where:  $a_M$  = activity of the specific element;  $a_C$  = activity of dissolved carbon; and  $P_{CO}^e$  = theoretical equilibrium partial pressure of carbon monoxide.

#### APPENDIX B

##### ACTIVITIES OF THE VARIOUS COMPONENTS OF INTEREST

$$a_C \text{ (activity of dissolved carbon)} = \%C \times f_C$$

$$f_C = f_C^C \times f_{Cr}^{Cr} \times f_{Ni}^{Ni} \times f_{Si}^{Si} \times f_{Mn}^{Mn}$$

$$\log f_C^C = 0.22 \times \%C$$

$$\log f_{Cr}^{Cr} = -0.024 \times \%Cr$$

$$\log f_{Ni}^{Ni} = 0.012 \times \%Ni$$

$$\log f_{Si}^{Si} = 0.106 \times \%Si$$

$$\log f_{Mn}^{Mn} = -0.012 \times \%Mn$$

$$a_{Cr} \text{ (activity of dissolved chromium)} = \%Cr \times f_{Cr}$$

$$f_{Cr} = f_{Cr}^C \times f_{Cr}^{Cr}$$

$$\log f_{Cr}^C = -0.12 \times \%C$$

$$\log f_{Cr}^{Cr} = 0$$

$$a_{Si} \text{ (activity of dissolved silicon)} = \%Si \times f_{Si}$$

$$f_{Si} = f_{Si}^C \times f_{Si}^{Si}$$

$$\log f_{Si}^C = 0.116 \times \%C$$

$$\log f_{Si}^{Si} = 0.112 \times \%Si$$

$$a_{Mn} \text{ (activity of dissolved manganese)} = \%Mn \times f_{Mn}$$

$$f_{Mn} = f_{Mn}^{Mn}$$

$$\log f_{Mn}^{Mn} = -0.0027 \times \%Mn$$

$$a_{Fe} \text{ (activity of iron)} = \text{Mole Fraction}$$

$$0.10 \leq a_{Cr} \leq 0.25$$

$$0.025 \times \%Mn \leq a_{Mn} \leq 0.05 \times \%Mn$$

$$0.03 \leq a_{Si} \leq 0.08$$

$$50 a_{FeO} = (0.125 \pm 0.025) \exp [-\%Ni + \%Cr/19.7]; 50\% \leq Fe \leq 100\%$$

where:  $f_C, f_{Cr}, f_{Si}, f_{Mn}$  represent the activity coefficients of carbon chromium, silicon and manganese respectively; and  $f_C^\alpha, f_{Cr}^\beta, f_{Si}^\gamma, f_{Mn}^\delta$  represent interaction parameters with superscripts

$$\alpha = C, Cr, Ni, Si, Mn$$

$$\beta = C, Cr$$

$$\text{and } \gamma = C, Si$$

60 The activities appropriate for nickel based alloys can be determined by the methods described in, for example; H. Schenck and M. G. Frohberg, *Steelmaking: The Chipman Conference*, The M.I.T. Press, Cambridge, Mass., 1963, and H. Schenck and E. Steinmetz, *Special Report No. 7, Stahleisen - Sonderberichte*, 1966, Publisher Stahleisen M.B.H., Dusseldorf.

65 The computer is programmed as shown in the logic diagram of FIG. 2 to select the lowest theoretical equi-

$$\Delta F^\circ =$$

$$C + O = CO(g)$$

$$-4,274 - 9.84T$$

librium partial pressure of carbon monoxide from which the computer then calculates the amount of carbon oxidized if all of the oxygen burns carbon and if not then the amount of carbon and metal oxidized. This is done by comparing the equilibrium partial pressure of CO with that which would be generated if all the oxygen burned carbon.

An alternate definition for the equilibrium partial pressure of CO is:

$$P_{CO}^e = F_{CO} P_s / F_{IG} + F_{CO} \quad (1)$$

Where:  $F_{CO}$  = flow of CO generated (an unknown);  $F_{IG}$  = flow of inert gas introduced;  $P_s$  = system pressure. If all of the oxygen burns carbon, the CO partial pressure can be calculated simply from the following equation:

$$P_{CO} = (2F_0/2F_0 + F_{IG})P_s \quad (2)$$

Where:  $F_{O_2}$  = flow of oxygen introduced. Now then, if the lowest selected  $P_{CO}^e \geq P_{CO}$  calculated from the equation directly above with all parameters known, then only carbon will be oxidized and in the amount  $C = 2F_{O_2} \times 12/387$ ;

Where:  $C$  = pounds of carbon oxidized per unit time, 12 is the molecular weight of carbon and 387 is the molar volume in cubic feet at 70° F and one atmosphere pressure.

On the other hand, should the lowest selected  $P_{CO}^e$  be less than  $P_{CO}$ ; then the amount of carbon burned is calculated directly from Equation (1) as follows:

$$P_{CO}^e = (F_{CO}/F_{CO} + F_{IG}) P_s$$

multiplying out  $P_{CO}^e F_{CO} + P_{CO}^e F_{IG} = F_{CO} P_s$  rearranging  $F_{CO} (P_s - P_{CO}^e) = P_{CO}^e F_{IG}$ ; then

$$F_{CO} = (P_{CO}^e F_{IG}/P_s - P_{CO}^e)$$

and in terms of pounds of carbon per unit time reduces to  $C = (P_{CO}^e / P_s - P_{CO}^e) F_{IG} 12/387$

The remainder of the oxygen, then, must oxidize metal. This is derived from the following formula:

$$M = 2 Wm/387 V [2 F_{O_2} - (P_{CO}^e F_{IG}/P_s - P_{CO}^e)]$$

Where:  $M$  = pounds of the metal oxidized per unit time;  $Wm$  = molecular weight of the metal lb./lb. - mole;  $V$  = valence of the metal. The amount of metal oxidized is subtracted from the original total metal weight and the total weight of the oxide resulting is added to the slag. The weight of the carbon oxidized is also subtracted from the original metal mass and new composition percentages are calculated. The new composition and weight are stored in memory and used in place of the old composition and weight at the start of the next cycle.

In order to establish the most favored of all the possible reactions from thermodynamics, the temperature must be known. The heat generated or absorbed by the reactions is determined from thermodynamic data and from the heat of reactions given in Appendix C shown below. These are translated into temperature by dividing them by the combined heat capacities of the metal, the vessel and the slag. The heat capacity of the metal in the case of steel is taken to be

$$= 10.5 \text{ lb.cal/lb. mol}^{\circ}\text{C} / 54 \text{ lb./lb. mol} \times W \text{ lbs. metal}$$

$$= 0.195 W \text{ lb. cal}^{\circ}\text{C}$$

Where:  $W$  = total metal weight in pounds. The heat capacity of the vessel (mainly the refractory) is taken to be

$$= 0.27 W_r F \text{ lb. cal}^{\circ}\text{C}$$

Where:  $W_r$  = total working lining refractory weight in pounds and  $F$  = empirical factor for the portion of the refractory lining which participates in the heat capacity of the system. The heat capacity of the slag is taken to be

$$= 0.55 W_s \text{ lb. cal}^{\circ}\text{C}$$

Where:  $W_s$  = slag weight in pounds. Thus, the heat capacity for the system at steelmaking temperatures is  $\gamma = 0.195 W + 0.27 F W_r + 0.55 W_s \text{ lb. cal}^{\circ}\text{C}$

The factor  $F$  has been determined by trial and error methods of comparing actual heat data with program results. This factor is shown in FIG. 3 indicating the proper value to be used as a function of refractory weight. The refractory lining weight is known from the vessel design and the metal and slag weights are calculated at the end of each time interval.

## APPENDIX C HEAT OF REACTION FOR THE VARIOUS OXIDATION REACTIONS

|    |                                                                                                                                         | Heat of Reaction    |
|----|-----------------------------------------------------------------------------------------------------------------------------------------|---------------------|
| 35 | $\frac{1}{2}O_2 \text{ } 25^{\circ} \text{C} \rightleftharpoons \frac{1}{2}O_2 \text{ } 1650^{\circ} \text{C}$                          | 6,727 lb.cal/lb-mol |
|    | $\frac{1}{2}O_2 \text{ } 1650^{\circ} \text{C} \rightleftharpoons O \text{ } 1650^{\circ} \text{C}$                                     | -28,000             |
|    | $\frac{1}{2}O_2 \text{ } 25^{\circ} \text{C} \rightleftharpoons O \text{ } 1650^{\circ} \text{C}$                                       | -21,273             |
|    | $C \text{ } 1650^{\circ} \text{C} + O \text{ } 1650^{\circ} \text{C} \rightleftharpoons CO \text{ } 1650^{\circ} \text{C}$              | -4,275              |
|    | $C \text{ } 1650^{\circ} \text{C} + \frac{1}{2}O_2 \text{ } 25^{\circ} \text{C} \rightleftharpoons CO \text{ } 1650^{\circ} \text{C}$   | -25,548             |
|    | $3Cr \text{ } 1650^{\circ} \text{C} + O \text{ } 1650^{\circ} \text{C} \rightleftharpoons Cr_3O_4 \text{ } 1650^{\circ} \text{C}$       | -244,800            |
|    | $3Cr \text{ } 1650^{\circ} \text{C} + 2O \text{ } 25^{\circ} \text{C} \rightleftharpoons Cr_3O_4 \text{ } 1650^{\circ} \text{C}$        | -329,892            |
|    | $Si \text{ } 1650^{\circ} \text{C} + 2O \text{ } 25^{\circ} \text{C} \rightleftharpoons SiO_2 \text{ } 1650^{\circ} \text{C}$           | -139,350            |
|    | $Si \text{ } 1650^{\circ} \text{C} + O \text{ } 25^{\circ} \text{C} \rightleftharpoons SiO_2 \text{ } 1650^{\circ} \text{C}$            | -181,896            |
|    | $Mn \text{ } 1650^{\circ} \text{C} + O \text{ } 1650^{\circ} \text{C} \rightleftharpoons MnO \text{ } 1650^{\circ} \text{C}$            | -58,400             |
| 40 | $Mn \text{ } 1650^{\circ} \text{C} + \frac{1}{2}O_2 \text{ } 25^{\circ} \text{C} \rightleftharpoons MnO \text{ } 1650^{\circ} \text{C}$ | -79,673             |
|    | $Fe \text{ } 1650^{\circ} \text{C} + O \text{ } 1650^{\circ} \text{C} \rightleftharpoons FeO \text{ } 1650^{\circ} \text{C}$            | -28,900             |
|    | $Fe \text{ } 1650^{\circ} \text{C} + \frac{1}{2}O_2 \text{ } 25^{\circ} \text{C} \rightleftharpoons FeO \text{ } 1650^{\circ} \text{C}$ | -50,173             |

For the elements of interest in steelmaking, the temperature change per percent oxidation are

45 Carbon:  $T = 21.3 W^{\circ}\text{C}/\gamma$

Chromium:  $= 21.2 W^{\circ}\text{C}/\gamma$

Manganese:  $= 14.5 W^{\circ}\text{C}/\gamma$

Silicon:  $= 65 W^{\circ}\text{C}/\gamma$

and Iron:  $= 8.95 W^{\circ}\text{C}/\gamma$

Such temperature increases are calculated from the composition and metal weight information derived at the end of each reaction time interval. The inert gas introduced reduces the temperature in a similar manner. Where the inert gas is argon the sensible heat increase is:

$$Ar (25^{\circ}\text{C}) = Ar (1,650^{\circ}\text{C})$$

$$\Delta H = 8,072 \text{ lb.cal/lb. mol}$$

60 and the temperature change due to each cubic foot of argon introduced is:

$$\text{Argon } \Delta T = 20.9^{\circ}\text{C}/\Delta$$

Finally, the steady state heat loss of the system due to its surroundings, which occurs regardless of the reactions within the vessel, is determined by means of empirical data presented in FIG. 4. These data result from extensive trial and error comparison of computer cal-

culations and actual experience. The new temperature of the bath is calculated by summing the various contributions and is stored in memory in addition to the new composition and weight data to replace the previous conditions at the start of the preparatory next succeeding time interval.

Once the computer has computed the new bath composition and temperature a determination is made as to whether the ratio of oxygen to inert gas should be adjusted. This determination is made for each cycle, i.e., each time the computer interrogates the progress of the heat. As explained earlier, this should be done at intervals of less than 2 minutes apart to conform to the theoretical assumption of a single reaction predominating during such time interval. It should be understood that the computer interrogates the progress of a heat solely from initial conditions without feedback information from the vessel. Hence, the computer can be operated simultaneously during the actual decarburization of the molten mass or establish beforehand the optimum flow conditions for such decarburization. In addition, the computer can conduct the decarburization operation automatically or, alternatively, provide detailed instructions for controlling the operation manually through an operator. For a completely automatic operation, as shown in FIG. 1, the output of the computer 22 is fed into the actuator 30 which in turn regulates the gas flow controls 18 and 20 respectively. The automatic actuator 26 takes the digital output information from the computer and converts such information to appropriate analog electrical signal levels representing the new gas flow rates. The flow controllers 18 and 20 respectively, when set for automatic operation, will respond to the new levels thereby adjusting the ratio of gas flow in accordance with the computer command. Actuator 26 is manually preset to establish initial flow conditions. Maintaining accurate fractional ratios, however, between the flow of oxygen and the inert gas requires highly expensive and complex gas flow controller systems. In those instances where the tonnage of molten mass to be decarburized is small, a tradeoff is suggested between a totally optimized operation and the high cost of a totally automatic system. In such cases the gas flow controls may be simplified to permit merely whole number ratio adjustments such that, for example, the oxygen to inert gas flow ratios are varied only in a monotonically descending order such as: 4:1, 3:1, 2:1, 1:1, 1:2, etc. Here as well, manual operation by an operator in response to computer instructions would be preferred. The program would be run through the computer with the computer readout 24 providing detailed instructions as to when to make adjustment to the gas ratio. Instruction would be based upon selecting in sequence the next closest whole integer ratio although the computer can instruct the operator to skip the next closest ratio and go to a subsequent one or, of course, to maintain the same ratio.

The selection of each succeeding gas ratio is determined in the preferred embodiment illustrated in FIGS. 2 and 2a by comparing the amount of oxidation of a specific element during each time interval with a predetermined critical limit for such element. The selection may also be made based on alternative methods which will be discussed hereafter in connection with the simplified flow chart of FIG. 7.

In the case of low carbon iron the specific element of interest is iron and when using the criterion of limited

oxidation for switching, a limit of oxidation is established for each time interval by dividing the total number of time intervals by the maximum acceptable limit of oxidized iron after decarburization. The limit for each time interval need not be the same, e.g., a lower limit may be used for a first given number of intervals and the limit then raised for the remaining intervals.

In the case of nickel based alloys the specific element of interest may be any single element selected from the 10 group consisting of chromium, molybdenum and niobium. The limit of oxidation would be established as in the case of low carbon iron.

In the case of iron based alloys the specific element of interest may be either chromium, molybdenum or 15 manganese. The limit of oxidation would be established as in the case of low carbon iron.

In the case of stainless steel the specific element of interest is chromium and the limit of oxidation may be established as in case of low carbon iron or alternatively and preferably as taught in U.S. Pat. No. 3,046,107 issued July 24, 1962, in the name of Edward C. Nelson et al. As taught in such patent the volume oxygen percent injected in the bath is dictated by the following relationship which is intended to apply for steel 20 containing 3 to 30 percent chromium:

$$\text{Percent O}_2 = \sqrt{\frac{13,000}{[13,000/(\text{Percent Cr}/\text{Percent C antilog } \sqrt{13,800/T} - 8.46)] - 1}}$$

Percent O<sub>2</sub> = Amount O<sub>2</sub>/O<sub>2</sub> + Inert Gas =  $F_{O_2}/F_{O_2} + F_{IG}$   
30 Where: percent Cr is the lower limit of chromium content in weight percent at the end of a time interval; T is the temperature of the melt in °K at the end of a time interval; percent C is the percent of carbon in the melt at the end of a time interval; and percent oxygen is the oxygen volume percent for such time interval.

The above formula may also be used to directly calculate the percent O<sub>2</sub> that should be employed for the next time interval. This may be done merely by using for percent Cr the calculated chromium content in weight percent at the end of the time interval. This would then determine whether the preceding flow of oxygen should be changed and to what extent.

In order to converse refractory the temperature of the bath, for each given time interval, should not be 45 permitted to exceed a predetermined maximum value. Likewise, to prevent premature solidification the temperature of the bath should not be permitted to fall below a predetermined minimum value. Hence, the computer 22 following a subroutine in the logic flow 50 chart of FIG. 2 and 2a will override any command to alter the flow rate of oxygen and diluting gas should the temperature fall below a preestablished acceptable temperature band. A functional relationship exists between the carbon content of a heat and the temperature. An acceptable temperature band corresponding to discreet carbon levels can therefore be established for any given heat. FIGS. 5 and 6 are two examples of empirically established acceptable temperature bands for stainless steel. This invention should not be construed as limited to any specific acceptable temperature band.

If the temperature for a given carbon level lies below the acceptable band, the computer will direct the operator to ignore any instructions to effect a change in the gas flow control in response to excess oxidation of the element of interest and instead to cause an increase in temperature by heating the molten mass. Such instruc-

tion may take the form of command to reset the gas flow control to establish a given flow rate, which may be the same as the existing flow rate or one with a higher proportion of oxygen, in order to prolong or intensify the exothermic reactions occurring in the bath during such time interval thus providing additional heat. The process cycle will then be renewed and the new temperature again evaluated to determine whether it lies within the acceptable band. This will continue until the temperature has risen to or above the acceptable lower limit. Operation of the process in such manner in order to regulate temperature requires however, a tradeoff in increased metallic oxidation. An alternative method for increasing the temperature of the molten bath is to add a deoxidizer to the mass such as by the addition of one or a combination of the following: silicon, aluminum, manganese, ferrosilicon, ferrochromium and ferromanganese. The addition of a deoxidizer may be used in combination with the first procedure to achieve a quicker response.

If the temperature for a given carbon content lies above the acceptable band, the computer 22 will direct the operator to cool the heat. The preferred method of cooling the heat is by the addition of scrap. The added scrap material must obviously be compatible with the molten metal composition. In order to avoid piecemeal scrap addition until the bath has cooled to a point in the acceptable band it is preferable that the operator add scrap in accordance with the following formula:

$$S \text{ (scrap addition)} = [T - T_{max} + T_{min}/2] C$$

Where:  $T$  = temperature of bath in °K;  $T_{max}$  = maximum acceptable temperature at the carbon level of the bath in °K;  $T_{min}$  = minimum acceptable temperature at the carbon level of the bath in °K and  $C$  is a constant. Other fluid coolants may also be used such as steam and carbon dioxide. Another alternative method of cooling, which may be used in combination with the above, is to inhibit the flow of oxygen and diluting gas for a predetermined period of time.

Although temperature override as described above is desirable it is not critical in practicing the present invention. The process may be carried out to achieve optimum economics without holding the temperature to within a predetermined temperature band. When the process is used without compensating for temperature the program illustrated in the logic diagram of FIGS. 2 and 2a effectively reduces to that shown in FIG. 7 where the block labeled "criterion for changing gas flow control" would be equivalent to the block labeled "element of interest oxidized more than established limit." Moreover, it is possible for some common starting metal composition to determine starting flow conditions which for such compositions will not cause the temperature to fall outside acceptable limits.

The selection of each succeeding gas ratio may be determined as stated hereinbefore by alternative methods to yield substantially the same result as the preferred method described above. These alternative methods are based on information regarding the carbon content, the temperature and the processing time respectively which are regularly monitored and stored by the computer. Temperature override is not necessary for these methods which are schematically described in the flow sheet shown in FIG. 7. Each method is based on a different criterion for changing the gas flow control. In the method based on carbon content, discrete gas ratios

are predetermined to correspond to carbon content ranges. Thus, when the computer finds that the carbon content has progressed from one range into a different range, it will render an indication to that effect and signal the operator to switch into a corresponding gas ratio in the flow control sequence or may perform this function automatically. In the method based on temperature, discrete gas ratios are predetermined to correspond to certain bath temperature ranges. Thus, when the computer finds that the temperature has progressed from one temperature range into the next, it will render an indication to that effect and signal the operator to switch to the corresponding ratio in the gas flow control sequence. In the method based on time, discrete gas ratios are predetermined to correspond to certain time periods relating to periods of progress in the refining operation. Thus, after a certain time period has elapsed, the operator is ordered to switch to the next gas ratio in the sequence. In each of these methods, the computer issues a final printout indication that the refinement is complete based upon the calculation that the carbon content is below a predetermined level. However, operation of the process by such alternative methods may not render the optimized economics offered by the preferred embodiment.

Appended hereto is a number of illustrative examples of steelmaking computer readout instructions for manual control of the decarburization operation as well as a printout of a complete program for directing the operation of the computer.

## EXAMPLES

Grade: Pure iron, 15 tons

35

| Instructions: (Time)(min)* | O <sub>2</sub> Flow rate =<br>Ar Flow Rate | O <sub>2</sub> Flow<br>Rate (NCFH) |
|----------------------------|--------------------------------------------|------------------------------------|
| 40                         | 0-9                                        | 4:1                                |
|                            | 9-14                                       | 3:1                                |
|                            | 14-31                                      | 4:1                                |
|                            | 31-36                                      | 1:1                                |

  

| Analyses: | %C             | %Cr   | %Si  | %Mn  | Temp°F    |
|-----------|----------------|-------|------|------|-----------|
| 45        | Starting       | 0.44  | 0.21 | 0.30 | 0.05 2710 |
|           | Computed Final | 0.001 | 0.22 | 0.00 | 0.00 3064 |
|           | Actual Final   | 0.001 | 0.10 | 0.00 | 0.01 3082 |

Actual Treatment Time=34 min.

\*Gas ratios were switched at the times (min) mentioned above to obtain the aim carbon.

Grade: 436,17 tons

55

| Instructions: (Time)(min)* | O <sub>2</sub> Flow Rate +<br>Ar Flow Rate | O <sub>2</sub> Flow<br>Rate (NCFH) |
|----------------------------|--------------------------------------------|------------------------------------|
| 60                         | 0-17                                       | 3.0:1                              |
|                            | 17-22                                      | 3.2:1                              |
|                            | 22-29                                      | 3.4:1                              |
|                            | 29-48                                      | 1.7:1                              |
|                            | 48-50                                      | 1.0:1                              |

  

| Analyses: | %C             | %Cr  | %Si   | %Mn  | Temp°F     |
|-----------|----------------|------|-------|------|------------|
| 65        | Starting       | 0.50 | 16.99 | 0.01 | 0.35 2880  |
|           | Computed Final | 0.08 | 15.09 | 0.01 | 0.15 3250  |
|           | Actual Final   | 0.08 | 15.09 | 0.01 | 0.12 3200+ |

Actual Treatment Time=50 min.

\*Gas ratios were switched at these mentioned time in minutes to obtain the aim carbon.

| Instructions: (Time)(min)* | O <sub>2</sub> Flow Rate +<br>Ar Flow Rate | O <sub>2</sub> Flow<br>Rate (NCFH) |
|----------------------------|--------------------------------------------|------------------------------------|
| 0-26                       | 3:1                                        | 22,800                             |
| 26-34                      | 2:1                                        | 17,700                             |
| 34-47                      | 1:2                                        | 8,850                              |

5

| Analyses:      | %C   | %Cr   | %Si  | %Mn  | Temp°F |
|----------------|------|-------|------|------|--------|
| Starting       | 0.52 | 19.30 | 0.28 | 1.05 | 2768   |
| Computed Final | 0.05 | 16.30 | 0.08 | 0.50 | 3207   |
| Actual Final   | 0.05 | 16.45 | 0.09 | 0.60 | 3200+  |

10

Actual Treatment Time=44 min.

\*Gas ratios were switched at these mentioned time to obtain the aim carbon.

## PROGRAM

## 23 SHORT TON - STAINLESS STEEL

## Input Data Definition

## 1. Variable:

T = Starting Temperature °F

CR = % Starting Chromium

C = % Starting Carbon

C1 = % Final desired carbon aim

SI = % Starting Silicon

MN = % Starting Manganese

Ni = % Starting Nickel

M = Starting metal weight in lbs.

## 2. Fixed

B = System pressure (1 atm)

RW = refractory weight (working lining) in lbs.  
(40,000 lbs.)

F. factor for the portion of working lining which participates in the heat capacity of the system (0.5)

IM = Total numbers of steps during oxygen blow (5)

AR = Argon flow rates in NCFH during various steps  
(NCF is 70°F and 1 atm) (7,600, 8,850, 17,700)

OX = Oxygen flow rates in NCFH during various periods (22,800, 17,700, 8,850)

ARS = Argon flow rate in NCFH through shroud  
(1,200/two tuyeres)

HL = Steady state heat loss expressed as °C/min.

20

AP = Argon pressure in p.s.i.g.  
OP = Oxygen pressure in p.s.i.g.  
OT = Oxygen inlet temp °F  
AT = Argon inlet temp °F

To be established in the plant

40

FE = percent Iron

SIO2 = Oxide of Si

CR304 = Oxide of Cr

MNO = Oxide of Mn

FEO = Oxide of Fe

TO2 = Total cubic ft of Oxygen

TA = Total cubic ft of Argon

Z2 = Time of oxygen blow

AEFO = Activity of FeO

CRI = percent Start Chromium

AMNO = Activity of MnO

AR(I) = Argon correction for temperature and pressure

OX(I) = Oxygen correction for temperature and pressure

50

Z = Calculation time (3 secs)

PT = Print time in min.

ASIO<sub>2</sub> = Activity of SiO<sub>2</sub>

14

ACR304 = Activity of Cr<sub>3</sub>O<sub>4</sub>

SIW = Weight of Si in metal in lbs.

MNW = Weight of Mn in metal in lbs.

CRW = Weight of Cr in metal in lbs.

FEW = Weight of Fe in metal in lbs.

NIW = Weight of Ni in metal in lbs.

CBR = Carbon removed as CO in lbs.

CRR = Chromium oxidized in lbs.

SIR = Silicon oxidized in lbs.

MNR = Manganese oxidized in lbs.

FER = Iron oxidized in lbs.

TM = Total moles of metals

XFE = Mole fraction of iron

AKCR = Equilibrium constant of Chromium and carbon reaction

ACR = Activity of chromium

AC = Activity of carbon

PCR = Partial pressure of CO with respect to Chromium reaction

AKSI = Equilibrium constant of Silicon and carbon reaction

ASI = Activity of Silicon

PSI = Partial pressure of CO with respect to Silicon reaction

AKMN = Equilibrium constant of Mn and carbon reaction

AMN = Activity of Mn

PMN = Partial pressure of CO with respect to Mn reaction

AKFE = Equilibrium constant of Fe and C reaction

AFE = Mole fraction of Fe

PFE = Partial pressure of CO with respect to Fe reaction

A = Argon in ft<sup>3</sup>/min.O<sub>2</sub> = Oxygen in ft<sup>3</sup>/min.

ACTOX = percent Oxygen in mixture of oxygen and argon

L = Lb moles of metals

CALOX = percent Oxygen calculated by Nelson Griffing formula

ECB = Temp rise due to carbon oxidation in °C

ECR = Temp rise due to Cr oxidation in °C

EMN = Temp rise due to Mn oxidation in °C

ESI = Temp rise due to Si oxidation in °C

EFE = Temp rise due to Fe oxidation in °C

AHL = Temp drop due to heating of Argon in °C/min.

E = Temp rise of system in °C

TMIN &amp; TMAX define the temperature band

SW = Weight of slag

SSIO<sub>2</sub> = % SiO<sub>2</sub> in slag

SFEO = % FeO in slag

SCR304 = % Cr<sub>3</sub>O<sub>4</sub> in slag

SMNO = % MnO in slag

SCRAP = Amount of scrap to cool the bath

S = Amount of scrap at any instant

CS = Carbon in scrap in lbs.

SIS = Silicon in scrap in lbs.

MNS = Manganese in scrap in lbs.

CRS = Chromium in scrap in lbs.

FES = Iron in scrap in lbs.

60

65

AODNG

```

100 REAL MN,NI,M,MNR,MNW,MNO,NIW
110 DIMENSION AR(7),OX(7),ARS(7),HL(7)
120 DATA B,T,CR,C,C1,SI,MN,NI,M,RW,F
130&/1,2768,19.3,.52,.05,.28,1.04,9.75,46200,40000,.5/
140 DATA IM
150&/3/
160 DATA AR
170&/7600,3850,17700,0,0,0,0/
180 DATA OX
190&/22800,17700,8850,0,0,0,0/
200 DATA ARS
210&/1200,1200,1200,0,0,0,0/
220 DATA AP,AT,OP,OT
230&/160,60,160,60/
232 DATA HL
234&/1.5,1.67,1.9,0,0,0,0/
240 T=(T+460.)/1.8
250 FE=100-CR-C-MN-NI-SI
260 SI02=0
270 CR304=0
280 MNO=0
290 FEO=0
300 T02=0
310 TA=0
320 Z2=0
325 CR1=CR
330 SCRAP=0
340 PRINT," TIME TEMP %C %CR %FE %SI %MN CO P "
350 PRINT 18,Z2,(1.8*T-460),C,CR,FE,SI,MN,(B*760)
360 AMNO=.035*MN
370 AFEO=.14*EXP(-(NI+CR)/19.7)
400 I=1
410 GO TO 60
420 40 I=I+1
430 PRINT,Z2,C,T*1.8-460
440 60 CONTINUE
450 AR(I)=AR(I)*(((AP+14.8)/174.8)*(520/(AT+460)))+.5+ARS(I)
460 OX(I)=OX(I)*(((OP+14.8)/174.8)*(520/(OT+460)))+.5
470 Z=.05
480 PT=5
490 ASI02=.05
500 ACR304=.15
510 TIME=0
520 SIW=SI*M*.01
530 CW=C*M*.01
540 MNW=MN*M*.01
550 CRW=CR*M*.01
560 FEW=FE*M*.01
570 NIW=NI*M*.01
580 17 CONTINUE

```

## AODNG CONTINUED

590 CBR=0  
 600 CRR=0  
 610 SIR=0  
 620 MNR=0  
 630 FER=0  
 640 TM=C/12+SI/28+MN/54.93+CR/52+FE/55.85+NI/58.69  
 650 XFE=FE/(TM\*55.85)  
 660 AKCR=EXP10(-12420/T+3.15)  
 670 ACR=EXP10(ALOG10(CR)-.12\*C)  
 680 AC=EXP10(ALOG10(C)+.22\*C+.106\*SI-.012\*MN+.012\*NI-.024\*CR)  
 690 PCR=(AKCR\*(ACR304)+.25\*AC)/(ACR)+.75  
 700 AKSI=EXP10(-14300/T+3.15)  
 710 ASI=SI\*EXP10(.166\*C+.112\*SI)  
 720 PSI=(AKSI\*(ASI02)+.5\*AC)/(ASI)+.5  
 730 AKMN=EXP10(-11830/T+7.85)  
 740 AMN=EXP10(ALOG10(MN)-.0027\*MN)  
 750 PMN=(AKMN\*AMN0\*AC)/AMN  
 760 AKFE=EXP10(-5415/T+4.83)  
 770 AFE=XFE  
 780 PFE=(AKFE\*AFE0\*AC)/AFE  
 790 A=AR(I)/60  
 800 O2=0X(I)/60  
 805 ACTOX=100\*O2/(O2+A)  
 807 CALOX=(13000/(((CR1/C)\*(EXP10(13800/T-3.46)))-100)+.5  
 810 IF(PSI-PCR)27,27,29  
 820 27 IF(PSI-PMN)28,28,35  
 830 28 IF(PSI-PFE)14,14,16  
 840 14 CALL PC(PSI,O2,B,A,T,CBR)  
 850 SIR=28\*.5\*(O2\*2/387-CBR/12)  
 860 P=PSI  
 870 GO TO 22  
 880 29 IF(PMN-PCR)35,35,26  
 890 35 IF(PMN-PFE)15,15,16  
 900 15 CALL PC(PMN,O2,B,A,T,CBR)  
 910 P=PMN  
 920 MNR=54.93\*(O2\*2/387-CBR/12)  
 930 GO TO 22  
 940 26 IF (PFE-PCR)16,16,20  
 950 16 CALL PC(PFE,O2,B,A,T,CBR)  
 960 P=PFE  
 970 FER=55.85\*(O2\*2/387-CBR/12)  
 980 GO TO 22  
 990 20 CALL PC(PCR,O2,B,A,T,CBR)  
 1000 P=PCR  
 1010 CRR=52\*.75\*(O2\*2/387-CBR/12)  
 1020 22 CONTINUE  
 1030 M=M-(CBR+SIR+CRR+MNR+FER)\*2  
 1040 L=M/54  
 1050 ECB=Z\*CBR\*25548/(12\*(L\*10.5+F\*RW\*.27))  
 1060 ECR=Z\*CRR\*329892/(3\*52\*(L\*10.5+F\*RW\*.27))

A0DNG CONTINUED

1070 EMN=Z\*MNR\*79673/(55\*(L\*10.5+F\*RW\*.27))  
 1080 ESI=Z\*SIR\*181896/(28\*(L\*10.5+F\*RW\*.27))  
 1090 EFE=Z\*FER\*50173/(56\*(L\*10.5+F\*RW\*.27))  
 1110 AHL=8072\*A/(387\*(L\*10.5+F\*RW\*.27))  
 1120 E=ECB+ECR+ESI+EMN+EFE-Z\*(AHL+HL(I))  
 1130 CW=CW-CBR\*Z  
 1140 T=T+E  
 1150 SIW=SIW-SIR\*Z  
 1160 MNW=MNW-MNR\*Z  
 1170 CRW=CRW-CRR\*Z  
 1180 FEW=FEW-FER\*Z  
 1190 C=100\*CW/M  
 1200 IF(T-1900)61,61,65  
 1210 65 TMIN=1985.6-159.8\*C-116.6\*(C)<sup>1/2</sup>+2.14\*(C)<sup>3</sup>  
 1220 TMAX=2039-104.1\*C-52.29\*(C)<sup>1/2</sup>-183.4\*(C)<sup>3</sup>  
 1230 IF(T-TMAX)61,61,62  
 1240 62 S=((T-(TMAX+TMIN)/2)\*(L\*10.5+RW\*F\*.27))/(2\*340)  
 1250 CS=.0005\*S  
 1260 CRS=.1825\*S  
 1270 MNS=.015\*S  
 1280 SIS=.005\*S  
 1290 FES=((100-.05-18.25-8.5-1.5-.5)\*S)/100  
 1300 CW=CW+CS  
 1310 CRW=CRW+CRS  
 1320 MNW=MNW+MNS  
 1330 SIW=SIW+SIS  
 1340 FEW=FEW+FES  
 1350 T=T-((S\*340)/(L\*10.5+RW\*F\*.27))  
 1360 M=M+S  
 1370 SCRAP=SCRAP+S  
 1380 61 CONTINUE  
 1390 C=CW\*100/M  
 1400 CR=CRW\*100/M  
 1410 SI=100\*SIW/M  
 1420 MN=100\*MNW/M  
 1430 FE=100\*FEW/M  
 1440 NI=100\*NIW/M  
 1450 CR304=CR304+CRR\*Z\*1.4614  
 1460 SI02=SI02+SIR\*Z\*2.1391  
 1470 MNO=MNO+MNR\*Z\*1.2913  
 1480 FEO=FEO+FER\*Z\*1.2865  
 1490 T02=T02+02\*Z  
 1500 TA=TA+A\*Z  
 1510 Z2=Z2+Z  
 1520 TIME=TIME+Z  
 1540 TMIN=1985.6-159.8\*C-116.6\*(C)<sup>1/2</sup>+2.14\*(C)<sup>3</sup>  
 1550 IF(T-TMIN)8,8,63  
 1560 63 IF(ACTOX-CALOX)8,8,7  
 1570 7 IF(I-IM)40,8,8  
 1580 8 CONTINUE

## AODNG CONTINUED

```

1590 IF(C-C1)10,11,11
1600 11 CONTINUE
1610 IF(TIME-PT)33,34,34
1620 33 CONTINUE
1630 GO TO 17
1640 34 TIME=0
1650 PRINT 18,Z2,(1.8*T-460),C,CR,FE,SI,MN,(P*760)
1660 18 FORMAT(F6.1,I6,F7.3,2F7.2,2F6.2,I5)
1670 GO TO 17
1680 10 PRINT18,Z2,(1.8*T-460),C,CR,FE,SI,MN,(P*760)
1690 PRINT,TA,TO2,SCRAP
1700 SW=SI02+CR304+FE0+MNO
1710 SSI02=SI02*100/SW
1720 SFE0=FE0*100/SW
1730 SCR304=CR304*100/SW
1740 SMNO=MNO*100/SW
1750 PRINT," METAL SLAG CR304 FE0 MNO CAO SI02 "
1760 PRINT 38,M,SW,SCR304,SFE0,SMNO,CAO,SSI02
1770 38 FORMAT(I6,I6,F7.1,F5.1,3F6.1)
1780 9 STOP
1790 END
1800 SUBROUTINE PC(P,02,B,A,T,CBR)
1810 IF(P-(2*02*1.3*B/(2*02+A)))19,2,2
1815 19 IF(C-.15)1,17,17
1820 1 CBR=(A*12/387)*(P/(B-P))
1822 GO TO 97
1825 17 CBR=(A*12/387)*(P/(B*1.3-P))
1827 97 CONTINUE
1830 IF (CBR-((2*02/387)*12))3,3,2
1840 2 CBR=(2*02/387)*12
1850 3 RETURN
1860 END
1870*****

```

What is claimed is:

1. A process for making steel by refining a predetermined mass of molten metal having a composition comprising carbon and iron, said mass being contained within a refractory lined vessel having means for injecting oxygen and a diluting gas therein, and adjustable gas flow control means for varying the flow rate of the respective gases; said process comprising:

- a. setting said adjustable control means to establish a first flow rate greater than zero for said oxygen and a first flow rate for said diluting gas;
- b. utilizing a computer to carry out the following sequence of steps:

1. calculating a plurality of activity coefficients, from data corresponding to the initial flow rate setting of each gas respectively and from the initial composition, weight and temperature of said mass of metal, that define the thermodynamic ac-

55

tivities of each element in said mass as a function of the composition of said mass, each coefficient reflecting the activity of each element in terms of the percentage of said element and the dependency of said element on the percentage of the other elements in said mass, with the activity of iron being equal to its mole fraction, and wherein the activities of the oxides of each element have predetermined values;

60

2. calculating a theoretical equilibrium partial pressure of carbon monoxide for the oxidation reaction of each element by means of said coefficients at said given temperature;

65

3. calculating the absolute maximum partial pressure of carbon monoxide assuming all the oxygen injected reacted solely with the carbon;

4. comparing the absolute maximum partial pressure of carbon monoxide from (3) with the lowest theo-

- retical equilibrium partial pressure of carbon monoxide from (2);
5. make a determination as to whether the lowest theoretical equilibrium partial pressure has a magnitude greater than the absolute maximum partial pressure and from said determination if such theoretical partial pressure is greater than the absolute maximum partial pressure then further calculate using said first gas flow rates, the amount of carbon oxidized and a new metal analysis and temperature for the composition;
6. make a determination as to whether the lowest theoretical equilibrium partial pressure has a magnitude of less than such absolute maximum partial pressure and from said determination if such theoretical partial pressure is of a magnitude lower than the absolute maximum partial pressure then further calculate from the theoretical equilibrium partial pressure of carbon monoxide and from said first gas flow rates the amounts of carbon and metal oxidized, a new metal analysis and temperature for the composition;
7. providing an indication of said new carbon content in said mass;
8. comparing the amount of oxidation of a specific single element in said mass with a preestablished limit of oxidation for said specific element;
9. providing an indication for resetting said adjustable gas flow control means to increase the proportion of diluting gas should the amount of oxidation of said specific element be at least equal to said preestablished limit of oxidation;
- c. resetting said adjustable gas flow control means in accordance with the indication provided in step (9)
- d. repeating the sequence from step (1) at predetermined time intervals of less than two minutes until the carbon content indicated in step (7) has at least decreased to a predetermined content.

2. A process as defined in claim 1 wherein each predetermined time interval in step (d) is between 3 to 30 seconds.

3. A process as defined in claim 2 wherein said diluting gas is selected from one of the following gases; helium, neon, argon, krypton, nitrogen, xenon and mixtures thereof.

4. A process as defined in claim 3 wherein the theoretical equilibrium partial pressure of carbon monoxide for each element is calculated, utilizing the computer, in accordance with the following equations:

$$K = \exp \Delta F^\circ / -RT$$

(1)

$$K = a_M^{x/y} P_{CO}^e / a_M^{y/x} a_O^{x/y} a_C$$

(2)

Where:  $K$  = equilibrium constant,  $\Delta F^\circ$  = standard free energy of the reaction;  $T$  = temperature ( $^\circ$ K);  $R$  is the gas constant;  $M$  is any metallic element;  $C$  and  $O$  represent carbon and oxygen respectively;  $x$  and  $y$  are integers which represent the chemical formula of the metallic oxide in question.  $a_M$  = activity of the specific element;  $a_C$  = activity of dissolved carbon; and  $P_{CO}^e$  = theoretical equilibrium partial pressure of carbon monoxide.

5. A process as defined in claim 4 wherein the com-

puter is used to carry out the following additional steps prior to step (c);

10. selecting a temperature band, from a preestablished acceptable temperature band correlative with carbon content, at the carbon level from steps (5) and (6);

11. comparing the temperature of steps (5) and (6) with the selected temperature band of step (10);

12. providing an indication to heat said molten mass if such temperature lies below said selected temperature band; and

13. providing an indication to cool said molten mass if such temperature lies above said selected temperature band.

6. A process as defined in claim 5 wherein prior to step (c) said molten mass is heated in accordance with said step (12) by resetting said adjustable gas flow control means to establish a second flow rate with the proportion of oxygen to diluting gas being at least equal to said first flow rate setting and further comprises the steps of repeating the sequence from step (1) until the temperature from steps (5) and (6) lies within said selected temperature band.

7. A process as defined in claim 6 wherein prior to step (c) said molten mass is heated in accordance with step (12) by adding a deoxidizer to said molten mass and further comprises the steps of repeating the sequence from step (1) until the temperature from steps (5) and (6) lies within said selected temperature band.

8. A process as defined in claim 7 wherein said deoxidizer is selected from one of the following; silicon, aluminum, manganese, ferrosilicon, ferrochromium and ferromanganese.

9. A process as defined in claim 5 wherein prior to step (c) said molten mass is cooled in accordance with the indication provided in step (13) by inhibiting said flow of oxygen and diluting gas for a predetermined period of time and further comprises the steps of repeating the sequence from step (1) until the temperature from steps (5) and (6) lies within said selected temperature band.

10. A process as defined in claim 5 wherein prior to step (c) said molten mass is cooled in accordance with the indication provided in step (13) by adding a coolant and further comprises the steps of repeating the sequence from step (1) until the temperature from steps (5) and (6) lies within said selected temperature band.

11. A process as defined in claim 10 wherein said coolant is a solid scrap material.

12. A process as defined in claim 11 further comprising the step of calculating the amount of scrap material to be added in accordance with the following equation:

$$S = [T - (T_{max} + T_{min})/2] C$$

Where:  $S$  = scrap addition;  $T$  = temperature in  $^\circ$ K of the mass at the end of a predetermined time interval;  $T_{max}$  = upper temperature limit of said selected temperature range;  $T_{min}$  = lower temperature limit of said selected temperature range; and  $C$  is a proportionality coefficient.

13. A process as defined in claim 10 wherein said coolant is a fluid selected from one of the following; steam and carbon dioxide.

14. A process as defined in claim 5 wherein said spe-

specific element is iron and wherein the preestablished limit of oxidation for said specific element is a fixed limit for each predetermined time interval.

15. A process as defined in claim 5 wherein said composition in addition comprises chromium.

16. A process as defined in claim 15 wherein said composition in addition comprises silicon and manganese.

17. A process as defined in claim 16 wherein said composition in addition comprises nickel.

18. A process as defined in claim 15 wherein said composition in addition comprises nickel, molybdenum and niobium.

19. A process as defined in claim 16 wherein said specific element is chromium and wherein the limit of oxidation for each time interval is established in accordance with the following equation:

$$\text{Volume \% Oxygen} = \frac{F_{O_2}/F_{O_2} + F_{IG}}{\sqrt{2713,000/[\text{Percent Cr/Percent C}}}$$

$$\text{antilog}(13,800/T - 8.46)]^{-1}$$

Where:  $F_{O_2}$  = flow of oxygen;  $F_{IG}$  = flow of inert gas; Percent Chromium = limit weight percentage of chromium that should remain in the bath at the end of each time interval; Percent C = the percent carbon by weight at the end of each time interval; and at  $T$  = temperature in  $^{\circ}\text{K}$  at the end of each time interval.

20. A process as defined in claim 17 wherein said specific element is selected from the class consisting of chromium, molybdenum and niobium and wherein the limit of oxidation is predetermined for each element and for each predetermined time interval.

21. A process as defined by claim 5 wherein said adjustable control means includes a predetermined number of discrete settings arranged in a predetermined sequence with each setting defining a fixed ratio of oxygen to diluting gas, and wherein the output of the computer is connected to said adjustable control means for automatically advancing said means in accordance with step (c) from said initially set first position to the next consecutive position once the oxidation of the specific element of interest is at least equal to the limit of oxidation for said element.

22. A process for making steel by refining a predetermined mass of molten metal having a composition comprising carbon and iron, said mass being contained within a refractory lined vessel having means for injecting oxygen and a diluting gas therein, and adjustable gas flow control means having a predetermined number of discrete positions with each position defining a fixed ratio of gas flow between the respective gases; said process comprising:

- setting said adjustable control means to a first position for establishing a first gas flow rate for said respective gases;
- utilizing a computer to carry out the following sequence of steps:

- calculating a plurality of activity coefficients from data corresponding to the initial flow rate setting of each gas respectively and from the initial composition, weight and temperature of said mass of metal, that define the thermodynamic activities of each element in said mass as a function of the composition of said mass, each coefficient reflecting the activity of each element in terms of the percentage of said element and the dependency of said element on the percentage of the

other elements in said mass, with the activity of iron being equal to its mole fraction, and wherein the activities of the oxides of each element have predetermined values;

- calculating a theoretical equilibrium partial pressure of carbon monoxide for the oxidation reaction of each element by means of said coefficients at said given temperature;
- calculating the absolute maximum partial pressure of carbon monoxide assuming all the oxygen injected reacted solely with the carbon;
- comparing the absolute maximum partial pressure of carbon monoxide from (3) with the lowest theoretical equilibrium partial pressure of carbon monoxide from (2);
- make a determination as to whether the lowest theoretical equilibrium partial pressure has a magnitude greater than the absolute maximum partial pressure and from said determination if such theoretical equilibrium partial pressure is greater than the absolute maximum partial pressure then further calculate from said first gas flow rates, the amount of carbon oxidized and a new metal analysis and temperature for the composition;
- make a determination as to whether the lowest theoretical equilibrium partial pressure has a magnitude of less than such absolute maximum partial pressure and if such theoretical partial pressure is of a magnitude lower than the absolute maximum partial pressure then further calculate from the theoretical equilibrium partial pressure of carbon monoxide and from said first gas flow rates the amounts of carbon and metal oxidized, a new metal analysis and temperature for the composition;
- providing an indication of the remaining carbon level in said mass from steps (5) and (6);
- comparing the carbon level of step (7) with a plurality of carbon level ranges, each range corresponding to a discrete position of said adjustable gas flow control means;
- selecting one carbon level range from said plurality of ranges in which the carbon level of step (7) resides;
- providing an indication for setting said adjustable flow control means to a position corresponding to the range selected in step (9);
- setting said adjustable gas flow control means in accordance with the indication provided in step (10) and
- repeating the sequence from step (1) at predetermined time intervals of less than two minutes until the carbon level indicated in step (7) reaches pre-established final carbon level.

23. A process as defined in claim 22 wherein each predetermined time interval in step (d) is between 3 to 30 seconds.

24. A process as defined in claim 23 wherein said diluting gas is selected from one of the following gases; helium, neon, argon, krypton, nitrogen, xenon and mixtures thereof.

25. A process as defined in claim 24 wherein the theoretical equilibrium partial pressure of carbon monoxide for each element is calculated, utilizing the computer, in accordance with the following equations:

$$K = \exp \Delta F^\circ / -RT$$

(1):

$$K = a_M^{x/y} P_{CO}^e / a_{M_x}^{i/y} o_y a_c$$

(2)

Where:  $K$  = equilibrium constant,  $\Delta F^\circ$  = standard free energy of the reaction;  $T$  = temperature ( $^{\circ}$ K);  $R$  is the gas constant;  $M$  is any metallic element; C and O represent carbon and oxygen respectively;  $x$  and  $y$  are integers which represent the chemical formula of the metallic oxide in question.  $a_M$  = activity of the specific element;  $a_c$  = activity of dissolved carbon; and  $P_{CO}^e$  = theoretical equilibrium partial pressure of carbon monoxide.

26. A process as defined in claim 25 wherein said composition in addition comprises chromium.

27. A process as defined in claim 26 wherein said composition in addition comprises silicon and manganese.

28. A process as defined in claim 27 wherein said composition in addition comprises nickel.

29. A process as defined in claim 26 wherein said composition in addition comprises nickel, molybdenum and niobium.

30. A process for making steel by refining a predetermined mass of molten metal having a composition comprising carbon and iron, said mass being contained within a refractory lined vessel having means for injecting oxygen and a diluting gas therein, and adjustable gas flow control means having a predetermined number of discrete positions arranged in a predetermined sequence with each position defining a fixed ratio of gas flow between the respective gases, said process comprising:

- setting said adjustable gas flow control means to a first position for establishing a first gas flow rate for said respective gases;
- utilizing a computer to carry out the following sequence of steps:

1. calculating a plurality of activity coefficients, from data corresponding to the initial flow rate setting of each gas respectively and from the initial composition, weight and temperature of said mass of metal, that define the thermodynamic activities of each element in said mass as a function of the composition of said mass, each coefficient reflecting the activity of each element in terms of the percentage of said element and the dependency of said element on the percentage of the other elements in said mass, with the activity of iron being equal to its mole fraction, and wherein the activities of the oxides of each element have predetermined values;

2. calculating a theoretical equilibrium partial pressure of carbon monoxide for the oxidation reaction of each element by means of said coefficients at said given temperature;

3. calculating the absolute maximum partial pressure of carbon monoxide assuming all the oxygen injected reacted solely with the carbon;

4. comparing the absolute maximum partial pressure of carbon monoxide from (3) with the lowest theoretical equilibrium partial pressure of carbon monoxide from (2);

5

10

15

20

25

30

35

40

45

55

60

65

5. make a determination as to whether the lowest theoretical equilibrium partial pressure has a magnitude greater than the absolute maximum partial pressure and if such theoretical partial pressure is of a magnitude lower than the absolute maximum partial pressure then further calculate from said first gas flow rates, the amount of carbon oxidized and a new metal analysis and temperature for the composition;

6. make a determination as to whether the lowest theoretical equilibrium partial pressure has a magnitude of less than such absolute maximum partial pressure and if such theoretical partial pressure is of a magnitude lower than the absolute maximum partial pressure then further calculate from the theoretical equilibrium partial pressure of carbon monoxide and from said first gas flow rates the amounts of carbon and metal oxidized, a new metal analysis and temperature for the composition;

7. providing an indication to advance the setting of said adjustable gas flow control means upon the expiration of predetermined time intervals;

8. comparing the carbon level of steps (5) and (6) with a preestablished final carbon level;

c. advancing the setting of said adjustable gas flow control means to the next consecutive position in said sequence in accordance with the indication provided in step (7);

d. repeating the sequence from step (1) at predetermined time intervals of less than 2 minutes; and

e. terminating the process when the carbon level of steps (5) and (6) at least reaches said final carbon level.

31. A process as defined in claim 30 wherein each predetermined time interval in step (d) is between 3 and 30 seconds.

32. A process as defined in claim 31 wherein said diluting gas is selected from the following gases; helium, neon, argon, krypton, nitrogen, xenon and mixtures thereof.

33. A process as defined in claim 32 wherein the theoretical equilibrium partial pressure of carbon monoxide for each element is calculated, utilizing the computer, in accordance with the following equations:

$$K = \exp \Delta F^\circ / -RT$$

(1):

$$K = a_M^{x/y} P_{CO}^e / a_{M_x}^{i/y} o_y a_c$$

(2)

Where:  $K$  = equilibrium constant,  $\Delta F^\circ$  = standard free energy of the reaction;  $T$  = temperature ( $^{\circ}$ K);  $R$  is the gas constant;  $M$  is any metallic element; C and O represent carbon and oxygen respectively;  $x$  and  $y$  are integers which represent the chemical formula of the metallic oxide in question.  $a_M$  = activity of the specific element;  $a_c$  = activity of dissolved carbon; and  $P_{CO}^e$  = theoretical equilibrium partial pressure of carbon monoxide.

34. A process as defined in claim 33 wherein said composition in addition comprises chromium.

35. A process as defined in claim 34 wherein said composition in addition comprises silicon and manganese.

36. A process as defined in claim 35 wherein said composition in addition comprises nickel.

37. A process as defined in claim 34 wherein said composition in addition comprises nickel, molybdenum and niobium.

38. A process for making steel by refining a predetermined mass of molten metal having a composition comprising carbon and iron, said mass being contained within a refractory lined vessel having means for injecting oxygen and a diluting gas therein, and adjustable gas flow control means having a predetermined number of discrete positions with each position defining a fixed ratio of gas flow between the respective gases; said process comprising:

a. setting said adjustable control means to a first position for establishing a first gas flow rate for said respective gases;

b. utilizing a computer to carry out the following sequence of steps:

1. calculating a plurality of activity coefficients, from data corresponding to the initial flow rate setting of each gas respectively and from the initial composition, weight and temperature of said mass of metal, that define the thermodynamic activities of each element in said mass as a function of the composition of said mass, each coefficient reflecting the activity of each element in terms of the percentage of said element and the dependency of said element on the activity of the other elements in said mass, with the activity of iron being equal to its mole fraction, and wherein the activities of the oxides of each element have predetermined values;

2. calculating a theoretical equilibrium partial pressure of carbon monoxide for the oxidation reaction of each element by means of said coefficients at said given temperature;

3. calculating the absolute maximum partial pressure of carbon monoxide assuming all the oxygen injected reacted solely with the carbon;

4. comparing the absolute maximum partial pressure of carbon monoxide from (3) with the lowest theoretical equilibrium partial pressure of carbon monoxide from (2);

5. make a determination as to whether the lowest theoretical equilibrium partial pressure has a magnitude greater than the absolute maximum partial pressure and from said determination if such theoretical partial pressure is greater than the absolute maximum partial pressure then further calculate using first gas flow rates, the amount of carbon oxidized and a new metal analysis and temperature for the composition;

6. make a determination as to whether the lowest theoretical equilibrium partial pressure has a magnitude of less than such absolute maximum partial pressure and from said determination if such theoretical partial pressure is of a magnitude lower than the absolute maximum partial pressure then further calculate from the theoretical equilibrium partial pressure of carbon monoxide and from said first gas flow rates the

amounts of carbon and metal oxidized, a new metal analysis and temperature for the composition;

7. providing an indication of the remaining carbon level from steps (5) and (6);

8. comparing the temperature from steps (5) and (6) with a plurality of temperature ranges each range corresponding to a predetermined one of said discrete positions;

9. selecting the temperature range from said plurality of ranges in which said temperature from steps (5) and (6) resides;

10. providing an indication for resetting said adjustable gas flow control means in accordance with the temperature range selected in step (9);

15. c. setting said adjustable control means in accordance with the indication provided in step (10);

d. repeating the sequence from step (1) at predetermined time intervals of less than 2 minutes until the carbon level from steps (5) and (6) reaches a predetermined final level.

39. A process as defined in claim 38 wherein each predetermined time interval in step (d) is between 3 to 30 seconds.

40. A process as defined in claim 39 wherein said diluting gas is selected from the following gases helium, neon, argon, krypton, nitrogen, xenon and mixtures thereof.

41. A process as defined in claim 40 wherein the theoretical equilibrium partial pressure of carbon monoxide for each element is calculated, utilizing the computer, in accordance with the following equations:

$$K = \exp \Delta F^\circ / -RT$$

(1);

$$K = a_M^{x/y} P_{CO}^e / a_{M_x}^{y/x} a_y a_C$$

(2)

Where:  $K$  = equilibrium constant,  $\Delta F^\circ$  = standard free energy of the reaction;  $T$  = temperature ( $^\circ$ K);  $R$  is the gas constant;  $M$  is any metallic element;  $C$  and  $O$  represent carbon and oxygen respectively;  $x$  and  $y$  are integers which represent the chemical formula of the metallic oxide in question.  $a_M$  = activity of the specific element;  $a_C$  = activity of dissolved carbon; and  $P_{CO}^e$  = theoretical equilibrium partial pressure of carbon monoxide.

50. 42. A process as defined in claim 41 wherein said composition in addition comprises chromium.

43. A process as defined in claim 42 wherein said composition in addition comprises silicon and manganese.

44. A process as defined in claim 43 wherein said composition in addition comprises nickel.

45. A process as defined in claim 42 wherein said composition in addition comprises nickel, molybdenum and niobium.

\* \* \* \* \*

UNITED STATES PATENT OFFICE  
CERTIFICATE OF CORRECTION

Patent No. 3,816,720

Dated June 11, 1974

Inventor(s) E. F. Bauer, et al

It is certified that error appears in the above-identified patent  
and that said Letters Patent are hereby corrected as shown below:

Claim 19: 2713,000 should read "13,000"

Signed and sealed this 1st day of October 1974.

(SEAL)

Attest:

McCoy M. GIBSON JR.  
Attesting Officer

C. MARSHALL DANN  
Commissioner of Patents